

1,322,786.

H. J. HAON,  
COATED PRODUCT,  
APPLICATION FILED JAN. 28, 1916.

Patented Nov. 25, 1919.



Harry J. Haon Inventor

By his Attorney

Prindle, Wright & Small

# UNITED STATES PATENT OFFICE.

HARRY J. HAON, OF NEWBURGH, NEW YORK, ASSIGNOR TO DU PONT FABRIKOID COMPANY, OF WILMINGTON, DELAWARE, A CORPORATION OF DELAWARE.

## COATED PRODUCT.

1,322,786.

Specification of Letters Patent. Patented Nov. 25, 1919.

Application filed January 28, 1916. Serial No. 74,735.

*To all whom it may concern:*

Be it known that I, HARRY J. HAON, of Newburgh, in the county of Orange, and in the State of New York, have invented a 5 certain new and useful Improvement in Coated Products, and do hereby declare that the following is a full, clear, and exact description thereof.

My invention relates particularly to sheets 10 of coated materials, such as woven fabrics, artificial leather, paper and leather, but especially to coated artificial leather.

The object of my invention is to provide a coated fabric in the form of a sheet, which 15 is of such a nature that it may be readily caused to adhere to other surfaces. More particularly, the object of my invention is to provide a product of this character, which is especially useful in bookbinding, and to 20 which gold-leaf and paper may be readily caused to adhere. A further object of my invention is to provide a pyroxylin coated product which, under the influence of heat or water or some other solvent, becomes 25 readily adherent to substances or materials applied to the surface thereof.

While my invention is capable of being carried out in many different ways, for the purpose of illustration I shall describe only 30 one example thereof hereinafter.

In the drawings, the single figure shows the perspective view of a fabric treated according to my invention.

My invention may, for example, be carried 35 out as follows: Any suitable backing, which may be a woven fabric, paper, or leather, and which may or may not already have been coated with one or more coats of various materials, but which is preferably an 40 artificial leather formed on a woven fabric backing by applying one or more coats of a pyroxylin solution containing 10 oz. by weight of pyroxylin, 1 gal. of solvent, comprising 15% of amyl acetate and 85% of 45 wood alcohol or 50% amyl acetate and 50% benzene, and which may contain any suitable pigment, is provided with a top coating containing pyroxlyn 10 oz. by weight, 1 gal. of a solvent comprising 15% amyl acetate 50 and 85% wood alcohol or 50% amyl acetate and 50% of benzene, and one pound of a fish glue solution containing 50% of glue and 50% of water, to which may be added, if desired, one oz. of birch tar or some similar

essential oil to remove the odor of the fish 55 glue and give the product an odor the same as that of Russian leather. Any other suitable adhesive material may also be added to the composition in this coating either in addition to or in substitution for the fish 6 glue solution, as for example gums, such as sandarac and shellac. The coating or coatings above referred to may be applied in any suitable way, as for example, by the use of a doctor blade, rolling, brushing, or flowing, and the coating containing the adhesive material may be applied before or after embossing. A product made in this manner, will readily adhere to materials placed upon the same under the influence of heat or moisture or both. The coated product thus produced is especially suitable for use in bookbinding as gold-leaf will readily adhere to the same when applied by a lettering tool, which has been previously heated to a moderate degree in the usual way. It will also readily adhere to paper, as for example, a paper which is applied to the inner faces of the books over the edges of the material used to cover the book, and when water or 80 a water soluble adhesive has been applied to the surface at the points where it is to adhere to the paper.

While I have described my invention above in detail, I wish it to be understood 85 that many changes may be made therein without departing from the spirit of my invention.

I claim:

1. A coated product comprising a backing 90 having an outer coating containing a mixture of pyroxylin and an adhesive, portions of said adhesive being exposed at the surface of the coated product.

2. A coated product comprising a backing 95 having a coating containing a mixture of pyroxylin and an adhesive, adapted to become adherent under the influence of heat, portions of said adhesive being exposed at the surface of the coated product.

3. A coated product comprising a backing having a coating containing a mixture of pyroxylin and an adhesive, adapted to become adherent under the influence of heat from a lettering tool heated to the usual 100 temperature, portions of said adhesive being exposed at the surface of the coated product.

4. A coated product comprising a backing

- having a coating containing a mixture of pyroxylin and an adhesive, adapted to become adherent upon the application of water, portions of said adhesive being exposed at the surface of the coated product. 5
5. A coated product comprising a backing having a coating containing a mixture of pyroxylin and fish glue. 10
6. A coated product comprising a backing of woven fabric having a coating containing a mixture of pyroxylin and an adhesive. 15
7. A coated product comprising a backing of woven fabric having a coating containing a mixture of pyroxylin and an adhesive, adapted to become adherent under the influence of heat. 20
8. A coated product comprising a backing of woven fabric having a coating containing a mixture of pyroxylin and an adhesive, adapted to become adherent under the influence of heat from a lettering tool heated to the usual temperature, portions of said adhesive being exposed at the surface 25 of the coated product.
9. A coated product comprising a backing of woven fabric having a coating containing a mixture of pyroxylin and an adhesive, adapted to become adherent upon the application of water, portions of said adhesive being exposed at the surface of the coated product. 30
10. A coated product comprising a backing of woven fabric having an outer coating containing a mixture of pyroxylin and fish glue. 35
11. A coated product comprising a backing of woven fabric already provided with a pyroxylin coating and on top of the same
- having a coating containing pyroxylin and an adhesive. 4
12. A coated product comprising a backing of woven fabric already provided with a pyroxylin coating and on top of the same having a coating containing pyroxylin and an adhesive, adapted to become adherent under the influence of heat. 4
13. A coated product comprising a backing of woven fabric already provided with a pyroxylin coating and on top of the same 50 having a coating containing pyroxylin and an adhesive, adapted to become adherent under the influence of heat from a lettering tool heated to the usual temperature. 55
14. A coated product comprising a backing of woven fabric already provided with a pyroxylin coating and on top of the same having a coating containing pyroxylin and an adhesive, adapted to become adherent upon the application of water. 60
15. A coated product comprising a backing of woven fabric already provided with a pyroxylin coating and on top of the same having a coating containing pyroxylin and fish glue. 65
16. A coated product comprising a woven fabric backing having a surface coating containing a mixture of pyroxylin and an adhesive adapted to be made adherent either by the application of heat or water, portions 70 of said adhesive being exposed at the surface of the coated product.

In testimony that I claim the foregoing I have hereunto set my hand.

HARRY J. HAON.

Witnesses:

CHAS. E. MACSHANE,  
F. GERARD WOOD.